

## UNITED STATES PATENT OFFICE.

ARTHUR SAMUEL O'NEIL, OF SPRINGFIELD, ILLINOIS, ASSIGNOR, BY MESNE ASSIGNMENTS, TO WESTERN CARTRIDGE COMPANY, OF EAST ALTON, ILLINOIS, A CORPORATION OF DELAWARE.

## BULK PROPELLANT POWDER.

No Drawing.

Application filed January 26, 1922. Serial No. 531,914.

This invention relates to bulk shotgun powder and to a process of preparing such powder whereby certain characteristics and desirable qualities are imparted thereto.

5 Ordinary bulk powders of the class referred to are manufactured from low nitration cottons. This is necessary in order to insure the desired ballistics. If cottons of high nitration were used the powder would

10 burn too rapidly and produce dangerously high pressures at the breech, and an attempt to correct this difficulty by reducing the charge would result in reduced velocities. Cottons of low nitration and powder made 15 therefrom are relatively hygroscopic and deteriorate rapidly because of the moisture absorbed.

Attempts have been made heretofore to use cottons of high nitration in the production of powder by adding a percentage of 20 rosin or other resinous material to the composition. This expedient has not met with success, however, owing to the manner in which the resins burn and the resulting production of acid decomposition products.

It is the object of the present invention to provide a powder which is relatively non-hygroscopic, hard, and of the desired density, and generally free from the defects of 30 the common grades of powder heretofore in use.

A further object of the invention is the provision of a method of manufacturing powder of the character described and particularly to enable the manufacturer to utilize less expensive solvents than those heretofore used.

Other objects and advantages of the invention will be apparent as it is better understood by reference to the following specification in which the preferred embodiments of the invention are described.

In carrying out the invention, cottons of any nitration may be employed though those of high nitration are preferred because of the non-hygroscopic quality which they impart to the powder. The rapidity of combustion which otherwise excludes many of these cottons from use in the manufacture of powder is readily overcome by the use of a deterrent material, preferably wood flour. This flour is not ordinary wood pulp but is granular or amorphous in form as distin-

guished from fibrous pulp. Preferably the wood flour should be sufficiently fine to pass 55 a 30 mesh screen. The use of wood flour in the composition permits not only proper control of the rapidity of combustion, but also produces a powder of lower gravimetric weight, the density of which may be varied 60 at will by the use of different proportions in the mixture.

To insure complete combustion of the wood flour and the consequent production of a smokeless powder, it is preferable to include in the composition a proportion of a metallic nitrate, e. g., barium, potassium or sodium nitrate. The proportion of metallic nitrates is, of course, varied, depending upon the proportion of wood flour in the composition.

It may also be desirable to introduce during the process of granulation and before the grain has hardened, a proportion of a nitro-hydrocarbon, e. g., dinitrotoluene, nitronaphthalene, or dinitrobenzene. These ingredients have a certain ballistic value and may be advantageously used for this reason. They serve, moreover, as a waterproofing and hardening agent for the powder grains. 75 Thus, if the powder is made from high nitro-cottons it is doubly protected from moisture. The nitrohydrocarbon also serves as a deterrent, partially or wholly replacing the wood flour.

Powder prepared with compositions described has a more firm and harder grain than powders ordinarily found in the market. It is freer from liability to absorb moisture and is more readily used in loading 80 shells because the harder surfaced grains flow freely through the loading machines. It is more uniform in quality than ordinary powders and insures the preservation of proper ballistic relations.

100 The powder is prepared in a suitable still, equipped with mechanical stirring apparatus. The nature and speed of the stirring apparatus are determined by the size of the powder grain to be produced. At the top of the still a fume-tight charging door is provided and a vapor line leads from the top to a water condenser. A discharging door or valve at the bottom of the still permits removal of the charge to a suitable filtering or 105 centrifugal apparatus wherein the powder is

separated from liquid, containing barium nitrate or other oxygen-carrying compounds, which is returned to the still. The still and appurtenant apparatus do not differ materially from that commonly employed in powder-making operations, and therefore is not illustrated.

In preparing the powder, the following procedure is preferably followed, although the details may be varied. A weighed amount of nitro-cotton having the desired nitration is added to a water solution of barium or other nitrate, and wood flour in the suitable proportion depending on the desired characteristics of the powder is added to the mixture in the still. The mass is agitated until the ingredients are thoroughly commingled and a solvent, preferably commercial ethyl acetate, is run into the still under continuous agitation until the nitro-cotton is colloided. Other solvents such as amyl acetate, butyl acetate, methyl acetate, ether-alcohol or acetone may be employed. The cheaper solvents are preferred. Heretofore only amyl or butyl acetate have been used and the process herein described has the advantage of permitting the elimination of these relatively more expensive solvents.

The mass in the still is heated by means of the steam jacket to the temperature necessary to distill the solvent, e. g., 85° C., until the greater part of the solvent is removed and recovered. A suitable amount of a nitrohydrocarbon, preferably dinitrotoluene, is then introduced. Nitronaphthalene, dinitrobenzene, or in fact any nitrohydrocarbon the melting point of which is about or below 100° C., may be used in place of dinitrotoluene. After further agitation to ensure thorough mixing, the charge is cooled to about 50° C. to freeze the nitrohydrocarbon which has entered the soft grain and the charge is dropped into the filtering or centrifugal apparatus, and after separation of the solution is ready for the dry house. After drying, the powder is screened through a rotary screen of the desired mesh and loaded into suitable containers.

A typical example of a shotgun powder produced in accordance with the invention herein described has the following composition.

|                   |        |
|-------------------|--------|
| External moisture | 0.74   |
| Internal moisture | 0.50   |
| Ash               | 0.82   |
| Barium nitrate    | 3.56   |
| Dinitrotoluene    | 9.53   |
| Wood flour        | 2.43   |
| Nitrocellulose    | 82.42  |
|                   | 100.00 |

It is to be observed that this composition

is merely representative and is not to be taken as a limitation of the invention.

The advantages of the powder prepared as hereinbefore described are its relatively non-hygroscopic character and uniform combustion rate depending upon the particular proportions of the deterrent agents which are employed in the composition. The advantages of the process are similar and include also the possibility of using relatively cheap solvents. The non-hygroscopic quality results from the use of cottons of higher nitration than is usual in preparing powders and from the application of nitrohydrocarbons before the grain hardens. The rate of combustion is controlled by the added wood flour and the nitrohydrocarbon, and the latter material is useful, moreover, to insure a harder grain than is otherwise possible.

Coated military powders have been known heretofore in which a coating is applied to the finished grain after drying. The invention herein described is not a coated or impregnated powder. The nitrohydrocarbon when applied is a part of the powder composition which is introduced before the powder grain is completed. The introduction of nitrohydrocarbons in this manner results in a new powder of markedly superior qualities which may be imparted thereto whether the wood flour is or is not employed in the composition.

Various changes may be made in the ingredients, the proportions thereof and in the process of compounding the powder without departing from the invention or sacrificing any of the advantages thereof.

I claim:

1. A bulk propellant powder including in its composition a nitro-cotton of high nitration and a deterrent material to reduce the rate of combustion of the powder.

2. A bulk propellant powder including in its composition a nitro-cotton of high nitration and wood flour as a deterrent material to reduce the rate of combustion of the powder.

3. A bulk propellant powder including in its composition a nitro-cotton of high nitration, wood flour and an oxidizing agent adapted and proportioned to ensure combustion of the wood flour.

4. A bulk propellant powder including in its composition nitro-cotton, a deterrent material to reduce the rate of combustion of the nitro-cotton, and an oxidizing agent adapted and proportioned to ensure complete combustion of the deterrent material.

5. A bulk propellant powder including in its composition nitro-cotton, a deterrent material to reduce the rate of combustion of the nitro-cotton, and a metallic nitrate adapted and proportioned to ensure complete combustion of the deterrent material.

6. A bulk propellant powder including in its composition nitro-cotton, wood flour and an oxidizing agent adapted and proportioned to ensure complete combustion of the wood flour.
7. A bulk propellant powder including in its composition nitro-cotton, wood flour and a metallic nitrate adapted and proportioned to ensure complete combustion of the wood flour.
8. A bulk propellant powder including in its composition nitro-cotton, a deterrent material to reduce the rate of combustion of the nitro-cotton and a nitro-hydrocarbon adapted and proportioned to water-proof the powder.
9. A bulk propellant powder including in its composition nitro-cotton, a deterrent material to reduce the rate of combustion of the nitro-cotton, an oxidizing agent adapted to ensure complete combustion of the deterrent material and a nitrohydrocarbon adapted and proportioned to water-proof the powder.
10. A bulk propellant powder including in its composition nitro-cotton, wood flour and a nitrohydrocarbon adapted and proportioned to water-proof the powder.
11. A bulk propellant powder including in its composition nitro-cotton, wood flour, an oxidizing agent adapted and proportioned to ensure complete combustion of the wood flour and a nitrohydrocarbon adapted and proportioned to water-proof the powder.
12. A propellant powder including in its composition nitro-cotton, wood flour, a metallic nitrate adapted and proportioned to ensure complete combustion of the wood flour and a nitrohydrocarbon adapted and proportioned to water-proof the powder.
13. A bulk propellant powder including in its composition nitro-cotton and dinitrotoluene adapted and proportioned to water-proof the powder.
14. A bulk propellant powder including in its composition nitro-cotton of high nitration, wood flour and dinitrotoluene.
15. A process of manufacturing powder, which comprises colloiding a nitro-cotton of high nitration to which a proportion of a combustion deterrent material has been added in the presence of a solvent, evaporating the solvent and granulating the powder.
16. A process of manufacturing powder, which comprises colloiding a nitro-cotton of high nitration to which a proportion of a combustion deterrent material has been added in the presence of a solvent, evaporating the solvent, mixing a nitrohydrocarbon with the mass before granulation is complete, and subsequently drying the powder.
17. A process of manufacturing powder, which comprises colloiding a nitro-cotton of high nitration to which a proportion of a combustion deterrent material has been added in the presence of a solvent, evaporating the solvent, mixing a nitrohydrocarbon with the mass before granulation is complete, and subsequently drying the powder.
18. A process of manufacturing powder, which comprises colloiding nitro-cotton in a solvent, evaporating the solvent, mixing a nitrohydrocarbon with the mass before granulation is complete, and subsequently drying the powder.
19. A process of manufacturing powder, which comprises colloiding nitro-cotton in a solvent, evaporating the solvent, mixing dinitrotoluene with the mass before granulation is complete, and subsequently drying the powder.
20. A process of manufacturing powder, which comprises mixing nitro-cotton and a combustion deterrent material with a solution of a metallic oxidizing salt adapted to insure oxidation of the deterrent material, mixing a solvent with the mass to colloid the nitro-cotton, evaporating the solvent and drying the powder.
21. A process of manufacturing powder, which comprises colloiding a nitro-cotton of high nitration in ethyl acetate in the presence of an insoluble deterrent material, evaporating the solvent and drying the powder.
22. A process of manufacturing powder, which comprises colloiding a nitro-cotton of high nitration in ethyl acetate in the presence of an insoluble deterrent material, evaporating the solvent, introducing a nitrohydrocarbon before granulation is complete, and drying the powder.
23. A process of manufacturing powder, which comprises colloiding a nitro-cotton of high nitration in ethyl acetate in the presence of an insoluble deterrent material, evaporating the solvent, introducing dinitrotoluene before granulation is complete, and drying the powder.

In testimony whereof I affix my signature.

ARTHUR SAMUEL O'NEIL.